

# UNITED STATES PATENT OFFICE.

JOSEPH BRADDOCK, OF INDIANAPOLIS, INDIANA.

## IMPROVED VARNISH.

Specification forming part of Letters Patent No. 59,174, dated October 30, 1866.

*To all whom it may concern:*

Be it known that I, JOSEPH BRADDOCK, of Indianapolis, in the county of Marion and State of Indiana, have invented a new and useful Composition of Matter for Coating Leather, Canvas, Metals, Wood, &c.; and I do hereby declare that the following is a full, clear, and exact description of the same, reference being had to the specimens of the ingredients and composition herewith filed.

The following description will enable persons skilled in the arts to compound and prepare the composition.

Take of spirits of turpentine five ounces, add one and one-half ounce of gum asphaltum, and boil over fire until dissolved; then add two drams of carriage-varnish and two ounces of lard-oil, or a like quantity of benzine. The last two ingredients are introduced alternatively in reference to the use to which the combination varnish is to be applied. The oil is used

where the varnish is intended to be applied to leather, canvas, &c., and the benzine is substituted for the oil when it is intended to apply the varnish to wood, metals, &c.

The varnish is to be applied with a brush to any substance that may require it in the ordinary way, and it must be renewed as required.

What I claim as my invention, and desire to secure by Letters Patent, is—

A combination varnish compounded from the ingredients named, or their chemical equivalents, substantially in the manner and for the purpose set forth.

In testimony whereof I have signed my name to this specification in the presence of two subscribing witnesses.

JOSEPH BRADDOCK.

Witnesses:

R. L. WALPOLE,  
THOS. W. HARDING.